

# UNITED STATES PATENT OFFICE.

RICHARD LAMB, OF NEW YORK, N. Y.

## METHOD OF IMPREGNATING WOOD.

1,168,944.

Specification of Letters Patent.

Patented Jan. 18, 1916.

No Drawing.

Application filed February 17, 1915. Serial No. 8,896.

To all whom it may concern:

Be it known that I, RICHARD LAMB, a citizen of the United States, residing at New York city, State of New York, have invented 5 certain new and useful Improvements in Methods of Impregnating Wood; and I do hereby declare the following to be a full, clear, and exact description of the invention, such as will enable others skilled in the art 10 to which it appertains to make and use the same.

My invention relates to the impregnating of porous materials—such as felt, wood, etc. The methods heretofore used are, first the 15 Bethel process: filling the pores, cells or hollow spaces with the impregnating liquid to an unnecessary extent; second, the Lowry process: after saturation of the wood under pressure, subjecting the wood to the action 20 of a vacuum, which only imperfectly removes the superfluous impregnating material; third, the Rueping process: the wood is subjected to a compressed gas or air pressure, and while maintaining the pressure, injecting the impregnating liquid at a still 25 higher pressure, which when cut off permits the compressed gas or air, previously inserted, to eject the surplus impregnating material.

30 In comparison with previous methods the present invention has advantages. It is an improvement over the Bethel process in that it provides a cheap and efficient method of ejecting the surplus impregnating material 35 from the wood. It is an improvement over the Lowry process in that a vacuum alone is not an efficient medium to withdraw the surplus impregnating material. It is an improvement over the Rueping process in that 40 it is possible to use the Rueping process without sterilizing the wood with steam, a step recognized in the art as very advantageous in all cases, and absolutely necessary when treating green wood. While steam 45 can be used as a separate and preliminary treatment in the Rueping process it is declared by the inventor that the preliminary treatment of the material by steam is not necessary, but that in certain cases it can 50 also be made use of. It is not named as a step in the process in any of the claims. In the Rueping process it is necessary to provide and maintain a gas or air compressor. My invention sterilizes the wood and re- 55 quires no compressor.

As one example of the working of my in-

vention: first, subject the material to be impregnated for a certain time, say three hours, to steam, of 30 pounds per square inch pressure. Without decreasing the pressure 60 set the blow-off valve at say about 120 pounds per square inch pressure. Inject, under 100 pounds per square inch pressure the impregnating material heated about 250 degrees Fahrenheit temperature. This is 65 the temperature of saturated steam at 30 pounds per square inch pressure. Heating the creosote oil or impregnating material to 250 degrees Fahrenheit prevents the steam from condensing when coming in contact 70 therewith. Condensing of the steam would destroy the pressure of the steam. After pumping creosote oil into the hermetically sealed cylinder in which the wood has been placed, withdraw the oil. The steam pressure in the wood will eject the oil from the wood to an extent determinable by experiment, varying with different woods. Pressure above given can be varied as conditions 75 may direct. After the pressure is relieved, 80 the usual vacuum can be applied to assist in draining the wood of surplus impregnating material.

The effect of my invention can be explained as follows: The steam pressure opens 85 the pores and sterilizes the wood. While the pores are still open and the steam still under pressure, the impregnating material, which in many cases will be creosote oil, is injected under a greater pressure than the 90 steam pressure, and at a temperature as high as that of the steam. The impregnating material will be given a pressure sufficient to thoroughly impregnate the wood, coating its fiber, and by use of some materials making the fiber hygroscopic as well as treating same with a germicidal agent. On releasing the pressure, by withdrawing the impregnating material from the treating cylinder, the steam pressure within the wood will eject 100 the surplus impregnating material from the pores, leaving only such amount as is shown by results is necessary to properly protect the wood, thus saving for further use the surplus impregnating material ejected. 105

I claim:—

1. The method of impregnating wood and other porous materials, which consists in placing the material to be treated in a hermetically sealed cylinder, and subjecting 110 same to steam pressure, then under a greater pressure, and with as high a degree of heat

injecting the impregnating material into the material to be treated, then withdrawing the impregnating material from the cylinder, when the steam pressure will eject the surplus impregnating material from the material treated substantially as described.

2. The method of impregnating wood and other porous material, which consists in placing the material to be treated in a hermetically sealed cylinder and subjecting same to steam pressure, then under a greater pressure and with as high a degree of heat injecting the impregnating material into the

material to be treated, then withdrawing the impregnating material from the cylinder 15 when the steam pressure will eject the surplus impregnating material from the material treated, then producing a vacuum in the cylinder to assist in ejecting the surplus impregnating material substantially as described. 20

RICHARD LAMB.

Witnesses:

MARY W. WALLACE,  
LAURA E. SMITH.